

[54] HIGH PERFORMANCE TUBULARS FOR CRITICAL OIL COUNTRY APPLICATIONS AND IMPROVED PROCESS FOR THEIR PREPARATION

[75] Inventor: James B. Greer, Houston, Tex.

[73] Assignee: Lone Star Steel Company, Dallas, Tex.

[\*] Notice: The portion of the term of this patent subsequent to Oct. 19, 1999, has been disclaimed.

[21] Appl. No.: 387,793

[22] Filed: Jun. 14, 1982

#### Related U.S. Application Data

[63] Continuation-in-part of Ser. No. 261,919, May 8, 1981, Pat. No. 4,354,882.

[51] Int. Cl.<sup>3</sup> ..... C21D 9/08

[52] U.S. Cl. ..... 148/12 R; 148/12 F; 148/12.4; 148/36

[58] Field of Search ..... 148/2, 12 R, 12 F, 12.4, 148/36, 144

#### References Cited

##### U.S. PATENT DOCUMENTS

|           |         |                 |          |
|-----------|---------|-----------------|----------|
| 2,825,669 | 3/1958  | Herzog          | 148/36   |
| 3,992,231 | 11/1976 | Timmons         | 75/126 C |
| 4,226,645 | 10/1980 | Waid et al.     | 148/36   |
| 4,282,047 | 8/1981  | Yamagata et al. | 148/36   |
| 4,354,882 | 10/1982 | Greer           | 148/36   |

#### FOREIGN PATENT DOCUMENTS

|          |        |                      |          |
|----------|--------|----------------------|----------|
| 604069   | 8/1960 | Canada               | 148/36   |
| 2756191  | 7/1978 | Fed. Rep. of Germany | 148/36   |
| 55-97423 | 7/1980 | Japan                | 148/36   |
| 791884   | 3/1958 | United Kingdom       | 148/12 F |

#### OTHER PUBLICATIONS

Selcuk, "Specification of Steel for Producing Petroleum Tube by Extrusion," Metals Technology, May 1982, vol. 9, pp. 177-181.

Primary Examiner—Peter K. Skiff

Attorney, Agent, or Firm—Donald E. Degling

#### [57] ABSTRACT

A high performance carbon steel tubular for critical Oil Country applications and an improved process for its preparation are disclosed. The tubular is particularly adapted for use in deep wells where the tubular may be subjected to high pressure, wide temperature ranges, and/or corrosive environments, which may include hydrogen sulfide, carbon dioxide, and brine water, together with hydrocarbons. The process comprises forming a bloom from a modified 41XX killed steel, upset forging and piercing the steel bloom into a cylindrical extrusion billet, cold machining the inside and outside diameters of the extrusion billet to be concentric and cold machining the nose of the extrusion billet, reheating and extruding the billet to form an extruded shell, intercritically heat treating the shell, removing surface defects, cold working the tubular shell to finished dimensions, intercritically heat treating the sized tubular, and quenching and tempering the finished tubular.

23 Claims, No Drawings

**HIGH PERFORMANCE TUBULARS FOR  
CRITICAL OIL COUNTRY APPLICATIONS AND  
IMPROVED PROCESS FOR THEIR  
PREPARATION**

**BACKGROUND OF THE INVENTION**

This application is a continuation-in-part of application Ser. No. 261,919 filed May 8, 1981, now U.S. Pat. No. 4,354,882.

**1. Field of the Invention**

The present invention relates to tubulars for deep oil and gas wells and a process for the preparation of such tubulars. More particularly, the invention relates to tubulars, commonly known as Oil Country Tubular Goods (OCTG), for use in wells 15,000 to 35,000 feet deep, which may be subjected to high pressures, wide temperature ranges, and/or corrosive environments which may include hydrogen sulfide, carbon dioxide, and brine water along with hydrocarbons as constituents.

**2. Discussion of the Prior Art**

In recent years, work has been done to develop well tubulars having higher strength and better resistance to failure under severe stress and corrosive applications. This work was necessitated by the demand for tubulars suitable for use in deep wells in the range of 15,000 to 35,000 feet deep, where pressures and temperatures may exceed 15,000 psi and 250° F., respectively. In addition, the tubulars may be subjected to highly corrosive atmospheres containing large quantities of hydrogen sulfide ( $H_2S$ ), carbon dioxide ( $CO_2$ ), brine water, and/or associated hydrocarbons. Tubulars subjected to these conditions may fail in a matter of hours due to sulfide stress cracking.

The sulfide stress cracking characteristic of steel tubulars may be influenced by many factors, including the chemistry of the steel, the nature and amounts of alloying elements, the microstructure of the steel, the mechanical processing of the steel, and the nature of the heat treatment which may be provided.

Over the years, many attempts have been made to overcome the sulfide stress cracking problem in carbon steels, but prior to the present invention, no fully satisfactory solution has appeared.

The following patents illustrate the current state of the art.

A process for making seamless tubes using the so-called Pilger process, followed by reheating to forging temperatures (preferably in the neighborhood of 2100° F.), and subsequent finishing in a plug mill, reeler, and sizing mill, is shown in U.S. Pat. No. 1,971,829.

U.S. Pat. Nos. 1,993,842, 2,275,801, and 2,361,318 disclose casing in which the collapse resistance is increased by subjecting the casing to cold radial compression up to 2 percent or slightly greater.

U.S. Pat. No. 2,184,624 discloses a heat treatment above the upper critical point followed by slow cooling prior to cold drawing to improve the machining qualities of a tube.

U.S. Pat. No. 2,293,938 suggests a combination of cold working a hot-rolled tube in the range of 5 to 10 percent, followed by a heat treatment below the lower critical point to increase the collapse resistance and maintain ductility.

Another method for improving properties, such as collapse resistance, is shown in U.S. Pat. No. 2,402,383, which discloses sizing a tubular casing formed about 3

to 10 percent over size while at a temperature somewhat below the lower critical temperature in the range of 650° to 1000° F.

U.S. Pat. No. 2,825,669 seeks to overcome sulfide stress corrosion cracking in a low carbon (less than 0.20 C) composition by adding chromium and aluminum and heat treating in the range lying between  $Ac_1$  and  $Ac_3$  followed by an austenitizing heat treatment and an anneal. U.S. Pat. No. 2,825,669 also teaches that if the carbon is too high (e.g., above 0.20 C), the resistance to stress corrosion cracking is impaired.

Another approach to the stress corrosion problem in low carbon steel (0.10 to 0.25 C) by heat treating is disclosed in U.S. Pat. No. 2,895,861. In this patent, the steel is austenitized for about one hour, followed by air cooling. Thereafter, the steel is tempered above the  $Ac_1$  point for about one hour.

U.S. Pat. No. 3,655,465 discloses a two-stage heat treatment for oil well casing involving an intercritical heat treatment to produce not more than 50 percent of an austenite decomposition product upon cooling. Thereafter, the product is tempered below the lower critical point.

U.S. Pat. No. 3,992,231 shows still another approach to the problem of overcoming sulfide stress cracking in SAE 41XX steels. In this process, the steel is austenitized, quenched, and thereafter temperstressed at a temperature below the transformation temperature by quenching the inner surface of the heated tube.

U.S. Pat. No. 4,032,368 discloses a process for reducing the time and energy required to perform an intercritical anneal for hypoeutectoid steel.

In U.S. Pat. No. 4,040,872, a method for strengthening a hypoeutectoid steel is disclosed. This comprises rapidly heating the steel into the austenite range (1350° to 2000° F.), quenching it, and then providing substantial cold working below the lower critical temperature.

Finally, in U.S. Pat. No. 4,226,645, a well casing having improved hydrogen sulfide stress cracking resistance is proposed. This patent discloses a tubular formed from an aluminum-killed steel containing controlled amounts of molybdenum, vanadium, and chromium, which is heat treated by austenitizing in the range of 1550° to 1700° F., quenching, and then tempering at 1200° to 1400° F. to produce a maximum hardness of 35 Rockwell C.

Specifications for deep well tubulars have been prepared by the American Petroleum Institute and various users. Such specifications describe grades of tubulars having yield strengths of, for example, 80,000, 90,000, 95,000, 110,000, 125,000, and 140,000 psi. A typical chemical composition for a modified 41XX steel for a 90,000 psi grade is specified in Table I, below.

**TABLE I**

| Constituent | Min. % | Max. % |
|-------------|--------|--------|
| Carbon      | .20    | .35    |
| Manganese   | .35    | .90    |
| Chromium    | .75    | 1.50   |
| Molybdenum  | .15    | .75    |
| Nickel      | —      | .25    |
| Copper      | —      | .35    |
| Phosphorus  | —      | .04    |
| Sulfur      | —      | .04    |
| Silicon     | —      | .35    |

60  
65  
66  
67  
68  
69  
70  
71  
72  
73  
74  
75  
76  
77  
78  
79  
80  
81  
82  
83  
84  
85  
86  
87  
88  
89  
90  
91  
92  
93  
94  
95  
96  
97  
98  
99  
100  
101  
102  
103  
104  
105  
106  
107  
108  
109  
110  
111  
112  
113  
114  
115  
116  
117  
118  
119  
120  
121  
122  
123  
124  
125  
126  
127  
128  
129  
130  
131  
132  
133  
134  
135  
136  
137  
138  
139  
140  
141  
142  
143  
144  
145  
146  
147  
148  
149  
150  
151  
152  
153  
154  
155  
156  
157  
158  
159  
160  
161  
162  
163  
164  
165  
166  
167  
168  
169  
170  
171  
172  
173  
174  
175  
176  
177  
178  
179  
180  
181  
182  
183  
184  
185  
186  
187  
188  
189  
190  
191  
192  
193  
194  
195  
196  
197  
198  
199  
200  
201  
202  
203  
204  
205  
206  
207  
208  
209  
210  
211  
212  
213  
214  
215  
216  
217  
218  
219  
220  
221  
222  
223  
224  
225  
226  
227  
228  
229  
230  
231  
232  
233  
234  
235  
236  
237  
238  
239  
240  
241  
242  
243  
244  
245  
246  
247  
248  
249  
250  
251  
252  
253  
254  
255  
256  
257  
258  
259  
260  
261  
262  
263  
264  
265  
266  
267  
268  
269  
270  
271  
272  
273  
274  
275  
276  
277  
278  
279  
280  
281  
282  
283  
284  
285  
286  
287  
288  
289  
290  
291  
292  
293  
294  
295  
296  
297  
298  
299  
300  
301  
302  
303  
304  
305  
306  
307  
308  
309  
310  
311  
312  
313  
314  
315  
316  
317  
318  
319  
320  
321  
322  
323  
324  
325  
326  
327  
328  
329  
330  
331  
332  
333  
334  
335  
336  
337  
338  
339  
340  
341  
342  
343  
344  
345  
346  
347  
348  
349  
350  
351  
352  
353  
354  
355  
356  
357  
358  
359  
360  
361  
362  
363  
364  
365  
366  
367  
368  
369  
370  
371  
372  
373  
374  
375  
376  
377  
378  
379  
380  
381  
382  
383  
384  
385  
386  
387  
388  
389  
390  
391  
392  
393  
394  
395  
396  
397  
398  
399  
400  
401  
402  
403  
404  
405  
406  
407  
408  
409  
410  
411  
412  
413  
414  
415  
416  
417  
418  
419  
420  
421  
422  
423  
424  
425  
426  
427  
428  
429  
430  
431  
432  
433  
434  
435  
436  
437  
438  
439  
440  
441  
442  
443  
444  
445  
446  
447  
448  
449  
450  
451  
452  
453  
454  
455  
456  
457  
458  
459  
460  
461  
462  
463  
464  
465  
466  
467  
468  
469  
470  
471  
472  
473  
474  
475  
476  
477  
478  
479  
480  
481  
482  
483  
484  
485  
486  
487  
488  
489  
490  
491  
492  
493  
494  
495  
496  
497  
498  
499  
500  
501  
502  
503  
504  
505  
506  
507  
508  
509  
510  
511  
512  
513  
514  
515  
516  
517  
518  
519  
520  
521  
522  
523  
524  
525  
526  
527  
528  
529  
530  
531  
532  
533  
534  
535  
536  
537  
538  
539  
540  
541  
542  
543  
544  
545  
546  
547  
548  
549  
550  
551  
552  
553  
554  
555  
556  
557  
558  
559  
5510  
5511  
5512  
5513  
5514  
5515  
5516  
5517  
5518  
5519  
5520  
5521  
5522  
5523  
5524  
5525  
5526  
5527  
5528  
5529  
5530  
5531  
5532  
5533  
5534  
5535  
5536  
5537  
5538  
5539  
5540  
5541  
5542  
5543  
5544  
5545  
5546  
5547  
5548  
5549  
55410  
55411  
55412  
55413  
55414  
55415  
55416  
55417  
55418  
55419  
55420  
55421  
55422  
55423  
55424  
55425  
55426  
55427  
55428  
55429  
55430  
55431  
55432  
55433  
55434  
55435  
55436  
55437  
55438  
55439  
55440  
55441  
55442  
55443  
55444  
55445  
55446  
55447  
55448  
55449  
55450  
55451  
55452  
55453  
55454  
55455  
55456  
55457  
55458  
55459  
55460  
55461  
55462  
55463  
55464  
55465  
55466  
55467  
55468  
55469  
55470  
55471  
55472  
55473  
55474  
55475  
55476  
55477  
55478  
55479  
55480  
55481  
55482  
55483  
55484  
55485  
55486  
55487  
55488  
55489  
55490  
55491  
55492  
55493  
55494  
55495  
55496  
55497  
55498  
55499  
554100  
554101  
554102  
554103  
554104  
554105  
554106  
554107  
554108  
554109  
554110  
554111  
554112  
554113  
554114  
554115  
554116  
554117  
554118  
554119  
554120  
554121  
554122  
554123  
554124  
554125  
554126  
554127  
554128  
554129  
554130  
554131  
554132  
554133  
554134  
554135  
554136  
554137  
554138  
554139  
554140  
554141  
554142  
554143  
554144  
554145  
554146  
554147  
554148  
554149  
554150  
554151  
554152  
554153  
554154  
554155  
554156  
554157  
554158  
554159  
554160  
554161  
554162  
554163  
554164  
554165  
554166  
554167  
554168  
554169  
554170  
554171  
554172  
554173  
554174  
554175  
554176  
554177  
554178  
554179  
554180  
554181  
554182  
554183  
554184  
554185  
554186  
554187  
554188  
554189  
554190  
554191  
554192  
554193  
554194  
554195  
554196  
554197  
554198  
554199  
554200  
554201  
554202  
554203  
554204  
554205  
554206  
554207  
554208  
554209  
554210  
554211  
554212  
554213  
554214  
554215  
554216  
554217  
554218  
554219  
554220  
554221  
554222  
554223  
554224  
554225  
554226  
554227  
554228  
554229  
554230  
554231  
554232  
554233  
554234  
554235  
554236  
554237  
554238  
554239  
554240  
554241  
554242  
554243  
554244  
554245  
554246  
554247  
554248  
554249  
554250  
554251  
554252  
554253  
554254  
554255  
554256  
554257  
554258  
554259  
554260  
554261  
554262  
554263  
554264  
554265  
554266  
554267  
554268  
554269  
554270  
554271  
554272  
554273  
554274  
554275  
554276  
554277  
554278  
554279  
554280  
554281  
554282  
554283  
554284  
554285  
554286  
554287  
554288  
554289  
554290  
554291  
554292  
554293  
554294  
554295  
554296  
554297  
554298  
554299  
554300  
554301  
554302  
554303  
554304  
554305  
554306  
554307  
554308  
554309  
554310  
554311  
554312  
554313  
554314  
554315  
554316  
554317  
554318  
554319  
554320  
554321  
554322  
554323  
554324  
554325  
554326  
554327  
554328  
554329  
554330  
554331  
554332  
554333  
554334  
554335  
554336  
554337  
554338  
554339  
554340  
554341  
554342  
554343  
554344  
554345  
554346  
554347  
554348  
554349  
554350  
554351  
554352  
554353  
554354  
554355  
554356  
554357  
554358  
554359  
554360  
554361  
554362  
554363  
554364  
554365  
554366  
554367  
554368  
554369  
554370  
554371  
554372  
554373  
554374  
554375  
554376  
554377  
554378  
554379  
554380  
554381  
554382  
554383  
554384  
554385  
554386  
554387  
554388  
554389  
554390  
554391  
554392  
554393  
554394  
554395  
554396  
554397  
554398  
554399  
554400  
554401  
554402  
554403  
554404  
554405  
554406  
554407  
554408  
554409  
554410  
554411  
554412  
554413  
554414  
554415  
554416  
554417  
554418  
554419  
554420  
554421  
554422  
554423  
554424  
554425  
554426  
554427  
554428  
554429  
554430  
554431  
554432  
554433  
554434  
554435  
554436  
554437  
554438  
554439  
554440  
554441  
554442  
554443  
554444  
554445  
554446  
554447  
554448  
554449  
554450  
554451  
554452  
554453  
554454  
554455  
554456  
554457  
554458  
554459  
554460  
554461  
554462  
554463  
554464  
554465  
554466  
554467  
554468  
554469  
554470  
554471  
554472  
554473  
554474  
554475  
554476  
554477  
554478  
554479  
554480  
554481  
554482  
554483  
554484  
554485  
554486  
554487  
554488  
554489  
554490  
554491  
554492  
554493  
554494  
554495  
554496  
554497  
554498  
554499  
554500  
554501  
554502  
554503  
554504  
554505  
554506  
554507  
554508  
554509  
554510  
554511  
554512  
554513  
554514  
554515  
554516  
554517  
554518  
554519  
554520  
554521  
554522  
554523  
554524  
554525  
554526  
554527  
554528  
554529  
554530  
554531  
554532  
554533  
554534  
554535  
554536  
554537  
554538  
554539  
554540  
554541  
554542  
554543  
554544  
554545  
554546  
554547  
554548  
554549  
554550  
554551  
554552  
554553  
554554  
554555  
554556  
554557  
554558  
554559  
554560  
554561  
554562  
554563  
554564  
554565  
554566  
554567  
554568  
554569  
554570  
554571  
554572  
554573  
554574  
554575  
554576  
554577  
554578  
554579  
554580  
554581  
554582  
554583  
554584  
554585  
554586  
554587  
554588  
554589  
554590  
554591  
554592  
554593  
554594  
554595  
554596  
554597  
554598  
554599  
554600  
554601  
554602  
554603  
554604  
554605  
554606  
554607  
554608  
554609  
554610  
554611  
554612  
554613  
554614  
554615  
554616  
554617  
554618  
554619  
554620  
554621  
554622  
554623  
554624  
554625  
554626  
554627  
554628  
554629  
554630  
554631  
554632  
554633  
554634  
554635  
554636  
554637  
554638  
554639  
554640  
554641  
554642  
554643  
554644  
554645  
554646  
554647  
554648  
554649  
554650  
554651  
554652  
554653  
554654  
554655  
554656  
554657  
554658  
554659  
554660  
554661  
554662  
554663  
554664  
554665  
554666  
554667  
554668  
554669  
554670  
554671  
554672  
554673  
554674  
554675  
554676  
554677  
554678  
554679  
554680  
554681  
554682  
554683  
554684  
554685  
554686  
554687  
554688  
554689  
554690  
554691  
554692  
554693  
554694  
554695  
554696  
554697  
554698  
554699  
554700  
554701  
554702  
554703  
554704  
554705  
554706  
554707  
554708  
554709  
554710  
554711  
554712  
554713  
554714  
554715  
554716  
554717  
554718  
554719  
554720  
554721  
554722  
554723  
554724  
554725  
554726  
554727  
554728

molybdenum as shown, for example, in NACE Standard MR-01-75, ¶3.3.3. The specification provides for an inside-outside quench following an austenitizing treatment so as to result in at least 90 percent martensite in the as-quenched condition. After tempering, the final hardness is specified in the range of 18 through 25 Rockwell C. Any surface defects, such as inclusions, laps, seams, tears, or blow holes, are required to be removed by grinding or machining to provide a minimum wall thickness of at least 87.5 percent of the nominal wall thickness.

#### BRIEF SUMMARY OF THE INVENTION

The present invention resulted from applicant's efforts to produce a premium product which would meet or exceed the above specifications for a 90,000 psi minimum yield strength tubular, as well as other grades of similar tubulars, such as those having minimum yield strengths of 80,000, 95,000, 110,000, 125,000 and 140,000 psi.

A modified AISI 41XX steel is appropriate for the practice of the present invention. Preferably, applicant employs the composition range shown in Table II, below.

TABLE II

| Constituent | Min. % | Max. % | Typical %  |
|-------------|--------|--------|------------|
| Carbon      | 0.20   | 0.35   | 0.27       |
| Manganese   | 0.40   | 0.70   | 0.50       |
| Phosphorus  | —      | 0.010  | 0.005      |
| Sulfur      | —      | 0.010  | 0.005      |
| Silicon     | 0.20   | 0.40   | 0.25       |
| Copper      | —      | 0.35   | 0.15       |
| Chromium    | 0.75   | 1.20   | 0.90       |
| Molybdenum  | 0.20   | 0.60   | 0.20-0.60* |
| Nickel      | —      | 0.25   | 0.15       |
| Vanadium    | 0.06   | 0.15   | 0.08       |

\*Molybdenum content will vary with wall thickness.

The steel is refined, preferably in an electric arc furnace using a double slag process, and continuously cast into blooms or billets having a substantially square cross section. In accordance with the present invention, the blooms are heated and upset forged in a cylindrical closed die and then pierced while in the die so as to form a pierced cylindrical extrusion billet. Thereafter the extrusion billet is fully machined on the inside diameter, outside diameter and the nose end is contoured. The machined extrusion billet is reheated and extruded to form a heavy wall extruded shell where the cross-sectional area of the extruded shell may be in the range of 10 to 40 percent over size with respect to the finished tubular. Following the extrusion step, in accordance with the invention, the extruded shell is subjected to an intercritical heat treatment by which the grain size of the material is refined. Thereafter, the heavy wall extruded shell is examined for defects and exterior defects are removed by contour grinding. In accordance with another feature of the invention, the shell thereafter is sized by substantial cold working. Following cold working, a second intercritical heat treatment is provided by the invention, as will be explained more fully below. Finally, the sized tubular is finished by a quench and temper process. Preferably, the quench is of the inside-outside type, particularly where heavy wall casting is involved. Typical tempering temperatures for the several grades of high performance tubulars are set forth in Table III, below.

TABLE III

| Yield Strength (psi) | Typical Tempering Temperature (°F.) |
|----------------------|-------------------------------------|
| 80,000               | 1300                                |
| 90,000               | 1275                                |
| 95,000               | 1265                                |
| 110,000              | 1235                                |
| 125,000              | 1200                                |
| 140,000              | 1165                                |

The finished tubular of the present invention is virtually defect-free, easily inspectable, and characterized by improved drift diameter. It has a closely controlled yield strength range with a correspondingly narrow range of hardness. The microstructure is characterized by a fine grain which is substantially tempered martensite, while the properties are characterized by an improved resistance to sulfide stress cracking, high toughness, and a high collapse strength.

#### DETAILED DESCRIPTION OF THE INVENTION

As shown in Table II, above, applicant has used relatively narrow ranges of chemical composition for his high performance tubulars for critical oil country applications. This composition has been selected so as to minimize alloy segregation while providing excellent hardenability and toughness. In order to achieve a high degree of cleanliness, it is preferable to refine the steel composition in an electric arc furnace using a double slag technique. Such a process is capable of producing closely controlled heats within the desired ranges of chemistry, including the very low levels of sulfur and phosphorus. The level of molybdenum depends upon tubular wall thickness, higher levels being used for greater wall thickness.

Although the refining technique is useful in achieving cleanliness, it is preferable to cast the finished heat by a continuous casting process rather than an ingot process, as the higher controlled cooling rates associated with continuous casting inhibit segregation in the bloom or billet.

It has been noted above that a fine grain structure is desirable in the finished tubular. This may more readily be attained if, at each step in the process, consideration is given to the effect of that process step on grain size and other properties. Thus, since applicant contemplates employing an extrusion process to prepare the extruded shell, the piercing step is the first point at which refining of the as-cast grain structure can begin and ultimate concentricity of the inside and outside finished walls affected. The substantially square cross section blooms produced by the continuous casting process are induction heated to about 2200° F. and upset forged in a cylindrical closed die to form a cylindrical extrusion billet. While still in the die the billet is pierced in the area which will become the tubular I.D. Preferably glass is used as a lubricant and oxidation barrier during the upset-pierce and subsequent extrusion operations. The forged and pierced billet is then cooled.

To improve concentricity, applicant machines the blooms or billets to produce a true cylindrical external surface which is free from scale and then bores a concentric internal diameter. With the establishment of concentric inside and outside surfaces, the bloom or billet may, if desired, be forged to expand the inside diameter prior to extrusion. The nose of the extrusion billet is also specially contoured by machining prior to

extrusion. Such machining accomplishes defect removal of potential laps and seams and assures maximum concentricity of the tubular following the subsequent extrusion step. The upset forging step provides an initial refining of the as-cast grain structure.

Applicant prepares the tubular form, preferably by an extrusion or similar process to form an extruded shell. During the hot forming extrusion process, considerable forging or working is accomplished with a corresponding refinement of the grain structure through additional distortion of the original as-cast grain structure. The extrusion process, however, has a particular advantage in the present invention. Surface defects, which may still remain in the extrusion billet or which may be introduced during processing, will appear as elongated axially-located defects on the surface of the extruded shell. Because the defects are positioned axially instead of helically on the surface of the tubular form (as occurs in the rotary piercing process), they can more easily be removed by contour grinding.

Following extrusion, applicant performs an intercritical heat treatment followed by defect removal. For steel compositions containing about 0.30 percent C, the lower critical temperature ( $Ac_1$ ) is about 1375° F., while the upper critical temperature ( $Ac_3$ ) is about 1500° F. Below the  $Ac_1$  point, the composition comprises pearlite and ferrite, while between the  $Ac_1$  and  $Ac_3$  points, the composition comprises austenite and ferrite. Above the  $Ac_3$  point, the composition is entirely austenitic. Within the intercritical range, the ratio of ferrite and austenite depends on the temperature under equilibrium conditions: at close to 1500° F. (for a steel containing 0.30 percent C), the composition is almost entirely austenite with only small amounts of ferrite. On the other hand, at 1375° F., the composition will contain ferrite as the major component. Thus, the temperature at which the intercritical heat treatment is performed determines the ratio between ferrite and austenite. On the other hand, the time of the heat treatment is not significant so long as sufficient time is allowed for the extruded shell to attain a uniform temperature so as to approximate equilibrium conditions. Intercritical heat treatment times in the range of 15 minutes to one hour are contemplated for an extruded shell having a wall thickness in the range of  $\frac{1}{2}$  to 1 inch.

Applicant has discovered that the intercritical heat treatment should be carried out at a point preferably just below the  $Ac_3$  point, i.e., at about 1475° F., for steels having a carbon content of about 0.30 percent. At this temperature, the grain structure will tend to recrystallize as relatively smaller grains. Following the intercritical heat treatment, cooling may be accomplished by any convenient manner, as such cooling is not critical.

In accordance with a further feature of the invention, the extruded shell, initially extruded so as to be 10 to 40 percent over size, is then cold worked to specified size. This cold working may be accomplished by Pilgering, rolling, swaging, or drawing, although cold working over a mandrel is preferred. Where the subsequent cold working is in excess of 10 percent, a significant degree of grain size refinement, after heat treatment, can occur. Preferably, the cold working during this step of the process is on the order of 20 percent so that a substantial degree of grain size refinement can be accomplished. This results in increased toughness and improved sulfide stress cracking resistance, properties significant in high pressure deep well tubulars.

Cold working to size after removal of surface defects by grinding produces another improved effect. Particularly where the cold working is performed over a mandrel, the process tends to "iron-out" or smooth out the contour ground surface so as to reduce the average depth of the ground area. Where cold working of about 20 percent is accomplished, original ground areas as deep as 30 percent of the wall thickness can be reduced to less than 5 percent of the nominal wall thickness. This has an additional advantage in that, from a fracture mechanics analysis, the toughness requirement for the product is decreased when the defect depth is reduced.

It will be appreciated that, where a mandrel is involved in the cold working process, surface irregularities on the interior surface of the tubular tend to be "ironed-out" as well as those on the exterior surface. This produces a smooth and highly inspectable product. In addition, the cold working over a mandrel process permits a closer control from end to end of the inside and outside diameters of the tubulars and the roundness of the tubulars. These characteristics are interrelated and improve the quality of the tubulars in several respects. First, the reduction in wall thickness variation resulting from the elimination or reduction of contour ground areas increases the collapse strength of the tubulars. Second, the improved control over wall thickness, roundness, and concentricity (resulting from reduced defect depth) permits the tubulars to be manufactured closer to the tolerance limits for the inside and outside diameters, thereby increasing the drift diameter of the tubulars. API drift is defined as: Nominal OD-2t-size tolerance, where OD=Outside Diameter and t=wall thickness.

Following the cold working to size step, preferably accomplished by cold working over a mandrel, applicant provides a second intercritical heat treatment wherein the sized tubular is again brought to a temperature between  $Ac_1$  and  $Ac_3$ . At this time, the grain structure has been substantially distorted because of the cold working and contains strains generally along the slip planes of each grain. During the intercritical heat treatment, recrystallization occurs from an increased number of nucleation sites created by the cold working process and thereby further refines the structure. Due to the relatively low intercritical temperature, grain growth is inhibited. The time for the heat treatment is not critical, provided that sufficient time is provided for complete recrystallization. For tubulars having wall thicknesses ranging from  $\frac{1}{2}$  to 1 inch, times in the range of 15 minutes to one hour at temperature are acceptable.

As noted above, quench and temper steps are performed as final processing steps. Preferably, the sized tubular is soaked at a temperature in the range of 1650° to 1700° F. for the minimum time required to assure complete austenitization. This, in turn, minimizes grain growth. Where the wall thickness of the tubular is more than  $\frac{1}{2}$  inch, it is preferable to use an inside-outside water quench to assure that substantially complete transformation of the austenite to martensite occurs. Preferably, the temperature of the tubular after quenching is held to a maximum of 200° F.

After the quench, the tubular is heat treated to a tempered martensite structure at a temperature below  $Ac_1$  to produce the required yield strength and hardness. For 80,000 to 140,000 psi yield strength materials, the tempering temperature generally will be in the range of 1100° to 1350° F.

As will be appreciated by those skilled in the art, it may be found desirable to straighten the tubular at one or more points in the process. Straightening may be performed by processes such as the well-known rotary straightening process.

In order to disclose more clearly the nature of the present invention, the following examples illustrating the invention are given. It should be understood, however, that this is done solely by way of example and is intended neither to delineate the scope of the invention nor limit the ambit of the appended claims. In the examples which follow, and throughout the specification, the quantities of material are expressed in terms of parts by weight, unless otherwise specified. Examples 1 and 2 demonstrate the improvement in sulfide stress cracking resistance developed in accordance with the process of the present invention while Examples 3 and 4 demonstrate the improvement in quality and dimensional control (e.g., the improvement in wall thickness uniformity which provides improved drift) resulting from the fully machined extrusion billet.

#### EXAMPLES 1 AND 2

(Heats 63920 and 73355)

Tubulars were produced which bracketed the 90,000 to 105,000 psi yield strength range for a 90,000 psi minimum yield strength grade using two distinct manufacturing processes:

- (1) Extrude, Q&T Heat Treatment
- (2) Extrude, (Normalize) Intercritical Heat Treatment—Draw Over Mandrel—Intercritical Heat Treatment, Q&T Heat Treatment.

The first of these processes corresponds to a standard method of manufacture for this grade tubular where a hot formed tube is heat treated to the proper strength range. The second process includes the applicant's intercritical heat treatment and cold working steps described herein, but is otherwise identical, as described below. Tube samples from each of these processes were tested according to the NACE TM-01-77 standard test method for characterization of their resistance to failure by sulfide stress cracking.

Heats having chemistries as shown in Table IV, below, were prepared in an electric arc furnace using a double slag process and continuously cast into 12,486-inch modified square blooms for piercing and extrusion.

TABLE IV

| Constituent | Heat 63910 | Heat 73355 |
|-------------|------------|------------|
| 5           | Carbon     | 0.30       |
|             | Manganese  | 0.57       |
|             | Phosphorus | 0.016      |
|             | Sulfur     | 0.021      |
|             | Silicon    | 0.25       |
|             | Copper     | 0.24       |
|             | Chromium   | 1.20       |
|             | Molybdenum | 0.54       |
|             | Nickel     | 0.14       |
|             | Tin        | 0.012      |
| 10          | Vanadium   | 0.096      |
|             | Aluminum   | 0.004      |

15 The blooms were pierced and then extruded to a diameter of 7.8 inches on two occasions. First, to assess the efficiency of the martensitic transformation upon quenching, tubulars were extruded for nominal 7 $\frac{5}{8}$  inch OD having 0.500 and 1.200 inch wall thicknesses. These tubulars were austenitized for about 45 minutes at 1675° F. and simultaneously inside and outside water quenched to 200° F. maximum. The tubulars were tempered at about 1250° and 1300° F. for about one hour to produce the range of yield strength shown in Table V. 20 The tempered tubulars were cooled with a water spray. Table V also shows the results of sulfide stress cracking tests performed on these tubulars.

25 Next, tubular shells were extruded as 7 $\frac{5}{8}$  inch OD and 0.712 inch wall thickness from blooms from the same two heats previously used. The extruded shells were subjected to an intercritical heat treatment of 1475° F. for about 20 minutes with slow cooling through the transformation range, followed by contour grinding of the OD scores, etc. The extruded and conditioned shells 30 are drawn over a mandrel to produce a 7-inch OD tube having a wall thickness of 0.625 inch. Such drawing represented a reduction in area of about 20 percent. Thereafter, a second intercritical heat treatment was performed at 1475° F. for 20 minutes and cooled slowly 35 through the transformation range.

40 These tubulars were austenitized for about 45 minutes at 1675° F. and simultaneously inside and outside water quenched to 200° F. maximum. The austenitized and quenched tubulars were tempered at about 1285° for 45 minutes and cooled with a water spray. Table VI shows the results of tubes 35 and 41 from this trial processing run. These tubes were selected because tube 41 had received a 1700° F. normalizing treatment just prior to the first intercritical heat treatment while tube 35 did 45 not receive the normalizing treatment.

TABLE V

SULFIDE STRESS CRACKING DATA FOR EXTRUDED AND QUENCH AND TEMPERED HEAT TREATED TUBULARS

| Sample Description         | Approximate Yield Strength, psi | Applied Stress, psi/Exposure Time, Hours |        |        |        |        |        |
|----------------------------|---------------------------------|------------------------------------------|--------|--------|--------|--------|--------|
|                            |                                 | 95,000                                   | 90,000 | 85,000 | 80,000 | 75,000 | 70,000 |
| <u>Heat 73355</u>          |                                 |                                          |        |        |        |        |        |
| 7 $\frac{5}{8}$ " x 0.500" | 91,500                          | —                                        | (12.4) | 720 NF | 720 NF | (217)  | —      |
| Tube No. 59                |                                 |                                          |        |        | 720 NF | 720 NF | 720 NF |
| 7 $\frac{5}{8}$ " x 1.200" | 88,500                          | —                                        | (33)   | (624)  | 720 NF | 720 NF | 720 NF |
| Tube No. 38                |                                 |                                          |        |        |        | 720 NF | 720 NF |
| 7 $\frac{5}{8}$ " x 1.200" | 105,000                         | (13.1)                                   | (26)   | 720 NF | 720 NF | 720 NF | 720 NF |
| Tube No. 55                |                                 |                                          |        |        |        |        | 720 NF |
| <u>Heat 63920</u>          |                                 |                                          |        |        |        |        |        |
| 7 $\frac{5}{8}$ " x 0.500" | 91,000                          | —                                        | —      | —      | 720 NF | 720 NF | 720 NF |
| Tube No. 57                |                                 |                                          |        |        |        | 720 NF | 720 NF |
| 7 $\frac{5}{8}$ " x 1.200" | 86,000                          | —                                        | (41.6) | 720 NF | 720 NF | 720 NF | 720 NF |

TABLE V-continued

SULFIDE STRESS CRACKING DATA FOR EXTRUDED AND QUENCH  
AND TEMPERED HEAT TREATED TUBULARS

| Sample Description | Yield Strength, psi | Approximate Applied Stress, psi/Exposure Time, Hours |        |        |        |        |        |
|--------------------|---------------------|------------------------------------------------------|--------|--------|--------|--------|--------|
|                    |                     | 95,000                                               | 90,000 | 85,000 | 80,000 | 75,000 | 70,000 |
| Tube No. 39        |                     |                                                      |        |        |        | 720 NF |        |

() Exposure time in hours at failure.

720 NF - Test completed to 720 hour exposure time without failure.

TABLE VI

SULFIDE STRESS CRACKING DATA FOR EXTRUDED,  
INTERCRITICAL HEAT TREATED -  
DRAWN OVER MANDREL-INTERCRITICAL HEAT TREATED,  
Q&T HEAT TREATED TUBULARS

| Sample Description | Yield Strength, psi | Approximate Applied Stress, psi/Exposure Time, Hours |        |        |        |        |         |
|--------------------|---------------------|------------------------------------------------------|--------|--------|--------|--------|---------|
|                    |                     | 95,000                                               | 90,000 | 85,000 | 80,000 | 75,000 | 70,000  |
| Heat 73355         |                     |                                                      |        |        |        |        |         |
| 7" X 0.625"        | 94,900              | (36.1)                                               | (16.7) | 720 NF | 720 NF | 720 NF | 720 NF  |
| Tube No. 35        |                     |                                                      |        | 720 NF | 720 NF | 720 NF | 720 NF  |
|                    |                     |                                                      |        | 720 NF | 720 NF | 720 NF | 720 NF  |
| 7" X 0.625"        | 100,200             | (7.5)                                                | 720 NF | 720 NF | 720 NF | (28.3) | 720 NF  |
| Tube No. 41        |                     |                                                      | 720 NF | 720 NF | 720 NF | 720 NF | 620 NF* |

() - Exposure time in hours at failure.

720 NF - Test completed to 720 hour exposure time without failure.

\*620 NF - Test terminated by severe weather at laboratory.

A comparison of the sulfide stress cracking results for the tubes manufactured by the conventional and new processes with all other conditions controlled as nearly identical as possible may be made using the data shown in Tables V and VI. Table V, for the conventional process, shows a threshold stress (no failure in 720 hours exposure time) for the two heats and wall thicknesses of 80,000 to 85,000 psi applied stress. Table VI shows a definite improvement in threshold stress to 85,000 to 90,000 psi applied stress. In both tables, an anomalous failure at 75,000 psi is noted. Since time-to-failure ordinarily shortens appreciably for higher stresses, an examination of the overall data trend indicates that an experimental error is likely for these two specimens. In this accelerated laboratory test, a commonly-accepted passing threshold stress is 75 percent of specified minimum yield strength, or 67,500 psi for this grade. Although both processes would be considered as passing these requirements, the increase in threshold stress for the new process is considered significant since passing tests at 90,000 psi applied stress are not common. No significant difference is noted between tube 41 from the new process described herein and tube 35 which received an additional normalizing step prior to the first intercritical heat treatment. The improvement in resistance to sulfide stress cracking shown by the data in Tables V and VI is felt to be the result of the intercritical heat treatment and cold working steps employed. Similar improvement would be expected for the new process over the conventional process for commensurately higher strength grades which are employed in less severe (for example, elevated temperature or lower hydrogen sulfide concentration) applications.

## EXAMPLES 3 AND 4

(Heats 73663, 73657, 73661A, and 73665)

Heats 73663 and 73657 (Example 3) were extruded from billets pierced in accordance with a prior art practice while Heats 73661A and 73665 (Example 4) were extruded from fully machined billets prepared in accor-

30 dance with the process of the present invention. Tables VII and VIII below contain measurements made on the extruded shells, Table VII contains the data for Heats 73663 and 73657, while Table VIII contains the data for Heats 73661A and 73665.

TABLE VII

| Extruded Shell Wall Eccentricity, As-Pierced Bore<br>(7.783" O.D. X 0.850" wall thickness extruded shell) |                |                           |           |
|-----------------------------------------------------------------------------------------------------------|----------------|---------------------------|-----------|
|                                                                                                           |                | Wall Eccentricity, Inches |           |
|                                                                                                           | Pipe No.       | Push End                  | Midlength |
| 40 Heat 73663                                                                                             | 1              | .051                      | .173      |
|                                                                                                           | 2              | .069                      | .104      |
|                                                                                                           | 3              | .058                      | .097      |
| 45 Heat 73657                                                                                             | Average        | .059                      | .125      |
|                                                                                                           | Std. Deviation | .009                      | .042      |
|                                                                                                           | 1              | .083                      | .077      |
|                                                                                                           | 2              | .067                      | .041      |
|                                                                                                           | 3              | .033                      | .054      |
|                                                                                                           | 4              | .104                      | .054      |
|                                                                                                           | 5              | .043                      | .143      |
|                                                                                                           | 6              | .053                      | .142      |
| 50                                                                                                        | 7              | .045                      | .098      |
|                                                                                                           | 8              | .061                      | .021      |
|                                                                                                           | Average        | .061                      | .079      |
|                                                                                                           | Std. Deviation | .023                      | .045      |

TABLE VII

| Extruded Shell Wall Eccentricity for ID Bored Billets<br>(7.783" O.D. X 0.805 wall thickness extruded shell) |          |                           |           |
|--------------------------------------------------------------------------------------------------------------|----------|---------------------------|-----------|
|                                                                                                              |          | Wall Eccentricity, Inches |           |
|                                                                                                              | Pipe No. | Push End                  | Midlength |
| 60 Heat 73661A                                                                                               | 1        | .017                      | .044      |
|                                                                                                              | 2        | .039                      | .028      |
|                                                                                                              | 3        | .045                      | .032      |
|                                                                                                              | 4        | .015                      | .035      |
|                                                                                                              | 5        | .034                      | .039      |
|                                                                                                              | 6        | .028                      | .038      |
|                                                                                                              | 7        | .077                      | .026      |
|                                                                                                              | 8        | .050                      | .048      |
|                                                                                                              | 9        | .023                      | .015      |
|                                                                                                              | 10       | .054                      | .056      |
| Average                                                                                                      |          | .038                      | .036      |
|                                                                                                              |          |                           | .035      |

TABLE VII-continued

Extruded Shell Wall Eccentricity for ID Bored Billets  
(7.783" O.D. x 0.805 wall thickness extruded shell)

| Pipe No.       | Wall Eccentricity, Inches |           |      |
|----------------|---------------------------|-----------|------|
|                | Push End                  | Midlength | Nose |
| Std. Deviation | .019                      | .012      | .010 |
| Heat 73665     |                           |           |      |
| 1              | .031                      | .039      | .016 |
| 2              | .029                      | .031      | .036 |
| 3              | .013                      | .016      | .029 |
| 4              | .027                      | .045      | .007 |
| 5              | .010                      | .017      | .045 |
| 6              | .017                      | .019      | .013 |
| 7              | .053                      | .031      | .025 |
| 8              | .027                      | .038      | .055 |
| 9              | .033                      | .018      | .052 |
| 10             | .017                      | .030      | .010 |
| 11             | .030                      | .015      | .025 |
| 12             | .035                      | .018      | .029 |
| 13             | .014                      | .018      | .020 |
| Average        | .026                      | .026      | .028 |
| Std. Deviation | .012                      | .010      | .015 |

Table IX below summarizes the measurements shown in Tables VII and VIII above.

TABLE IX

(Summary of Tables VII and VIII)

|                     | Average Wall Eccentricity (inches) | Standard Deviation ( $\sigma$ ) |
|---------------------|------------------------------------|---------------------------------|
| As Pierced          | .059                               | .009                            |
|                     | .125                               | .042                            |
|                     | .072                               | .038                            |
|                     | .061                               | .023                            |
|                     | .079                               | .045                            |
|                     | .040                               | .017                            |
| Grand Average       | .073                               | .029                            |
| % of Wall Thickness | 8.5%                               | 3.4%                            |
| Bored               | .038                               | .019                            |
|                     | .036                               | .012                            |
|                     | .035                               | .010                            |
|                     | .026                               | .012                            |
|                     | .026                               | .010                            |
|                     | .028                               | .015                            |
| Grand Average       | .032                               | .013                            |
| % of Wall Thickness | 3.7%                               | 1.5%                            |

As shown by Table IX, both the average values of the concentricity measurements and the standard deviations of those measurements are substantially larger for the extruded shells produced by the prior art piercing process than for those produced by the process of the present invention. These values may be translated into percent eccentricity values by reference to the nominal wall thickness of the extruded shells (0.850"). Thus the as pierced shells had an 8.5% eccentricity with a standard deviation of 3.4%, while the machined shells had a 3.7% eccentricity with a standard deviation of 1.5%. As the heats shown in Tables VII and VIII were run through the extruder consecutively in a single extrusion run, they include a constant value due to whatever misalignment may have been present in the extruder at that time. Thus, the relative improvement due to the present invention is greater than is suggested by these figures.

The terms and expressions which have been employed are used as terms of description and not of limitation, and there is no intention in the use of such terms and expressions of excluding any equivalents of the features shown and described or portions thereof, but it is recognized that various modifications are possible within the scope of the invention claimed.

What is claimed is:

1. A process for manufacturing high performance tubulars having minimum yield strengths ranging from 80,000 to 140,000 psi characterized by improved sulfide stress cracking resistance and improved dimensional control comprising the steps of providing a killed steel bloom comprising in amounts by weight 0.20 to 0.35 percent carbon, 0.35 to 0.90 percent manganese, 0.75 to 1.50 percent chromium, 0.15 to 0.75 percent molybdenum, 0.25 percent maximum nickel, 0.35 percent maximum copper, 0.040 percent maximum phosphorus, 0.04 percent maximum sulfur, 0.35 percent maximum silicon, and the balance iron, except normal steelmaking impurities, upset forging the killed steel bloom in a closed end cylindrical die to form an extrusion billet, hot piercing the extrusion billet while still in the upset forging die, cold machining the outside diameter and the inside diameter to be concentric and cold machining the nose of the extrusion billet, reheating and extruding the extrusion billet to form an extruded shell wherein the cross-sectional area of the extruded shell is in the range of 10 to 40 percent larger than the cross-sectional area of the finished tubular, subjecting the extruded shell to a first intercritical heat treatment to recrystallize and refine the grain structure, removing surface defects by grinding, sizing the ground, heat treated extruded shell by cold working to the finished tubular dimensions, subjecting the sized tubular to a second intercritical heat treatment to recrystallize and refine the grain structure, and subjecting the finished tubular to a quench and temper process wherein the tubular is austenitized, quenched, and tempered to produce a substantially tempered martensitic structure having a minimum yield strength in the range of 80,000 to 140,000 psi.
2. A process according to claim 1, in which the steel consists essentially in amounts by weight of from 0.20 to 0.35 percent carbon, 0.40 to 0.70 percent manganese, 0.20 to 0.40 percent silicon, 0.75 to 1.20 percent chromium, 0.20 to 0.60 percent molybdenum, 0.06 to 0.15 percent vanadium, and the balance iron, except normal steelmaking impurities.
3. A process in accordance with claim 1, in which the steel is refined in an electric arc furnace and continuously cast into blooms.
4. A process in accordance with claim 3 in which the refining step employs a double slag process to minimize the sulfur and phosphorus content of the steel.
5. A process in accordance with claim 1, in which the first intercritical heat treatment is performed by holding the extruded shell at a temperature in the range between the  $Ac_1$  and  $Ac_3$  temperatures for a period of 15 minutes to one hour.
6. A process according to claim 1, in which surface defects are removed by contour grinding.
7. A process according to claim 1, in which the ground heat treated extruded shell is cold worked to finished size by drawing said extruded shell over a mandrel.
8. A process according to claim 1, in which the second intercritical heat treatment is performed by holding the sized tubular at a temperature in the range between the  $Ac_1$  and  $Ac_3$  temperatures for a period of 15 minutes to one hour.
9. A process according to claim 2, in which the quench and temper process comprises an inside-outside water quench from a temperature in the austenitizing range of 1650° to 1700° F. to a temperature in the range of 100° to 200° F.

10. A process according to claim 2, in which the sized tubular is tempered at a temperature in the range of 1250° F. to 1350° to produce a yield strength range of 80,000 to 95,000 psi.

11. A process according to claim 2, in which the sized tubular is tempered at a temperature in the range of 1250° to 1325° F. to produce a yield strength range of 90,000 to 105,000 psi.

12. A process according to claim 2, in which the sized tubular is tempered at a temperature in the range of 1225° to 1300° F. to produce a yield strength range of 95,000 to 110,000 psi.

13. A process according to claim 2, in which the sized tubular is tempered at a temperature in the range of 1200° to 1275° F. to produce a yield strength range of 110,000 to 125,000 psi.

14. A process according to claim 2, in which the sized tubular is tempered in a temperature in the range of 1150° to 1250° F. to produce a yield strength range of 125,000 to 140,000 psi.

15. A process according to claim 2, in which the sized tubular is tempered at a temperature in the range of 1100° to 1200° F. to produce a yield strength range of 140,000 to 155,000 psi.

16. A process for manufacturing high performance tubulars having minimum yield strengths ranging from 80,000 to 140,000 psi characterized by improved sulfide stress cracking resistance and improved dimensional control, comprising the steps of providing a killed steel bloom consisting essentially in amounts by weight of from 0.20 to 0.35 percent carbon, 0.40 to 0.70 percent manganese, 0.20 to 0.40 percent silicon, 0.75 to 1.20 percent chromium, 0.20 to 0.60 percent molybdenum, 0.06 to 0.15 percent vanadium, and the balance iron, except normal steelmaking impurities, upset forging the killed steel bloom in a closed end cylindrical die to form an extrusion billet, hot piercing the extrusion billet while still in the upset forging die, cold machining the outside diameter and the inside diameter to be concentric and cold machining the nose of the extrusion billet, reheating and extruding the extrusion billet to form an extruded shell wherein the cross-sectional area of the

extruded shell is in the range of 10 to 40 percent larger than the cross-sectional area of the finished tubular, subjecting the extruded shell to a first intercritical heat treatment to recrystallize and refine the grain structure, removing surface defects by grinding, sizing the ground, heat treated extruded shell by cold working to the finished tubular dimensions, subjecting the sized tubular to a second intercritical heat treatment to recrystallize and refine the grain structure, and subjecting the finished tubular to a quench and temper process wherein the tubular is austenitized, quenched, and tempered to produce a substantially tempered martensitic structure having a minimum yield strength in the range of 80,000 to 140,000 psi.

17. A process according to claim 16, in which the sized tubular is tempered at a temperature in the range of 1250° to 1350° F. to produce a yield strength in the range of 80,000 to 95,000 psi.

18. A process according to claim 16, in which the sized tubular is tempered at a temperature in the range of 1250° to 1325° F. to produce a yield strength in the range of 90,000 to 105,000 psi.

19. A process according to claim 16, in which the sized tubular is tempered at a temperature in the range of 1225° to 1300° F. to produce a yield strength in the range of 95,000 to 110,000 psi.

20. A process according to claim 16, in which the sized tubular is tempered at a temperature in the range of 1200° to 125° F. to produce a yield strength in the range of 110,000 to 125,000 psi.

21. A process according to claim 16, in which the sized tubular is tempered at a temperature in the range of 1150° to 1250° F. to produce a yield strength in the range of 125,000 to 140,000 psi.

22. A process according to claim 16, in which the sized tubular is tempered at a temperature in the range of 1100° to 1200° F. to produce a yield strength in the range of 140,000 to 155,000 psi.

23. A high performance tubular made in accordance with the process set forth in any one of claims 1, 2, or 16.

\* \* \* \* \*

UNITED STATES PATENT AND TRADEMARK OFFICE  
CERTIFICATE OF CORRECTION

PATENT NO. : 4,394,189

Page 1 of 2

DATED : July 19, 1983

INVENTOR(S) : James Brison Greer

It is certified that error appears in the above-identified patent and that said Letters Patent are hereby corrected as shown below:

At column 2, line 48, "institute" should be --Institute--.

At column 4, line 14, "hardenss" should be --hardness--.

At column 5, line 53, "by" should be --in--.

At column 7, line 45, "12,486" should be --12.486--.

At column 8, line 35, "are" should be --were--.

At column 10, line 55, "Table VII" should be --Table VIII--.

At column 11, line 1, "Table VII" should be --Table VIII--.

At column 10, line 57, "0.805" should be --0.850"--.

At column 11, line 3, "0.805" should be --0.850"--.

UNITED STATES PATENT AND TRADEMARK OFFICE  
CERTIFICATE OF CORRECTION

PATENT NO. : 4,394,189

Page 2 of 2

DATED : July 19, 1983

INVENTOR(S) : James Brison Greer

It is certified that error appears in the above-identified patent and that said Letters Patent is hereby corrected as shown below:

At column 13, line 3, "1250°F to 1350°" should be --1250° to 1350°F--.

At column 13, line 18, "in a temperature" should be --at a temperature--.

At column 14, line, 29 "125°F" should be --1275°F--.

Signed and Sealed this  
Tenth Day of April 1984

[SEAL]

Attest:

GERALD J. MOSSINGHOFF

Attesting Officer

Commissioner of Patents and Trademarks